

## UNITED STATES PATENT OFFICE.

JOSEPH NÜSSLIN, OF LUDWIGSHAFEN-ON-THE-RHINE, GERMANY, ASSIGNEE TO  
I. G. FARBENINDUSTRIE AKTIENGESELLSCHAFT, OF FRANKFORT-ON-THE-MAIN,  
GERMANY, A CORPORATION OF GERMANY.

FULLING WOOL AND THE LIKE.

No Drawing. Application filed August 13, 1926, Serial No. 129,087, and in Germany January 21, 1925.

This application is a continuation in part including subject-matter transferred from my copending application Ser. No. 83,143, filed January 22nd, 1926, and has as its object an improved process for fulling wool or other animal fibres and preparations suitable for carrying out this process.

I have disclosed in my copending application Ser. No. 83,143 that operations or processes to which fibrous materials or textiles are subjected and in which no soap has been or can be used, can be improved by an addition of organic sulfonic acids or their salts to the preparations or liquids applied to the said materials. The sulfonic acids to be employed in accordance with my invention may belong to the aliphatic series such as sulfonated brown coal tar oils, or more suitably to the aromatic series. Among the latter, in general, those containing side chains have been found to be most suitable. I may mention as examples of compounds especially suitable for these purposes propyl and butyl derivatives of naphthalene sulfonic acids, also aromatic sulfonic acids substituted by alkylated amino groups, for example dimethyl metanilic acid, diethyl-alpha-naphthylamine sulfonic acid or similar compounds, or their salts.

The said sulfonic acids can be used with great advantage as an addition to acid fulling baths used for wool or other animal fibres. The sulfonic acids may be employed in connection with other additions, including soap or saponaceous materials. By the said additions the materials are very uniformly and rapidly wetted and well penetrated by the fulling bath. The ordinary process of acid fulling is objectionable for the reason that much time is necessary to complete the penetration of the fibres by the acid and further for the reason that due to the varying permeability of the walls of the fibre to the acid part of the fibre is fulled to a greater extent than the rest of it, producing an uneven effect. The beneficial action produced by applicant's addition of a very small amount of sulphonated acids of aromatic hydrocarbons is due in the main to the fact that such addition promotes a more ready and intimate contact between the walls and the acid solution owing to the high wetting and penetrating power of the sulphonated acid. By virtue of these properties the fulling process is effected far more

thoroughly and in a much shorter time than hitherto. Furthermore the difficulty arising from the varying permeability of the fibres is overcome, for the reason that by the use of these compounds the fibres are completely fulled at all points regardless of differences in permeability thus producing the desired even appearance. The sulfonic acids have the great advantage of being stable in acid solutions, whereby the necessity of using alkali fulling and subjecting animal fibres, especially wool, to the risk of being damaged by the alkali, is avoided. In the process of fulling which forms the subject matter of this application, care should, however, be taken to ascertain that the sulfonic acids employed possess in the utmost only weak tanning properties, which means that they should be practically unsuitable for use in tanning.

For example, acid fulling may be carried out at ordinary temperature with dilute sulfuric acid of 3 degrees Baumé, containing about 2 grammes of isopropylated naphthalene sulfonic acid or its salts per litre. The operation is effected with woolen goods, for example unfelted hat bodies, for about an hour whereupon the acid is washed out as usual.

It is to be understood that my invention is not limited to this particular example which is only given for the purpose of illustrating how my invention may be carried out in practice.

I do not generally claim, in this application, the processes of treating fibres or fibrous materials with the aid of sulfonic acids, as are claimed in the parent application Ser. No. 83,143.

What I claim is:

1. The process of acid fulling wool and other animal fibres comprising the step of treating with an acid bath containing less than one per cent of an aromatic sulfonic acid substituted by a side chain which is practically unsuitable for use in tanning.
2. The process of acid fulling wool and other animal fibres comprising the step of treating with an acid bath containing less than one per cent of naphthalene sulfonic acid substituted by an alkyl radicle selected from the group of propyl and butyl radicles.
3. An acid fulling bath for woolen goods containing less than one per cent of naphthalene sulfonic acid substituted by an

alkyl radicle selected from the group of propyl and butyl radicles in conjunction with an acid fulling agent.

4. As a composition for the acid-fulling of wool, sulphuric acid of 3 degrees Baume containing at least two grams per liter of an aromatic sulphonic acid substituted by a side chain.

5. The process of acid fulling wool and other animal fibres comprising the step of treating with an acid bath containing a small quantity of an aromatic sulphonic acid substituted by a side chain.

6. The process of acid fulling wool and

other animal fibres comprising the step of 15 treating with an acid bath containing a small quantity of naphthalene sulphonic acid substituted by an alkyl radicle selected from the group of propyl and butyl radicles.

7. An acid fulling bath for woolen goods 20 containing a small quantity of naphthalene sulphonic acid substituted by an alkyl radicle selected from the group of propyl and butyl radicles in conjunction with an acid fulling agent. 25

In testimony whereof I have hereunto set my hand.

JOSEPH NÜSSLEIN.